

## UNITED STATES PATENT OFFICE

JAMES D. LINDSAY, OF WHITING, INDIANA, ASSIGNOR TO STANDARD OIL COMPANY,  
OF WHITING, INDIANA, A CORPORATION OF INDIANA

## POLISH

No Drawing.

Application filed April 16, 1927. Serial No. 184,433.

This invention relates to polishes and particularly to a polish for automobile and other highly finished surfaces.

The polish comprises water, mineral oil, 5 finely divided colloidal earthy material, an abrasive and organic acids.

Any suitable mineral oil may be used. It is preferred to use a mineral oil such as straw oil together with a more viscous oil, such as 10 a lubricating oil of viscosity about 75-85 sec. Saybolt at 100° F. It is preferred to use a highly treated or white oil since results are somewhat better than when a less treated oil is employed.

15 As the colloidal earthy material, wilkinite, bentonite, precipitated silicic acid or similar highly colloidal clay is preferred. As the abrasive it is preferred to use suitable earthy abrasive materials, such as infusorial earth, 20 finely divided silica, or the like.

Various organic acids may be used such as oxalic, tartaric, acetic acid and other acids and hydroxy acids. It is, however, found 25 that better results are obtained by using a mixture of oxalic and tartaric acids.

A polish according to the invention may suitably contain the following ingredients in the percentages by weight stated: Water 56 30 to 71%, mineral oil 23 to 36%, wilkinite 0.2 to 0.5%, infusorial earth 3 to 6%, oxalic acid 1 to 1.5% and tartaric acid 1 to 1.5%.

The following composition is a highly satisfactory polish:

|                                        | Per cent |    |
|----------------------------------------|----------|----|
| Water                                  | 65       |    |
| Mineral seal oil                       | 19       |    |
| White oil (Vis. 75 Saybolt at 100° F.) | 9½       |    |
| Wilkinite                              | ¼        |    |
| Infusorial earth                       | 3¾       | 80 |
| Oxalic acid                            | 1¼       |    |
| Tartaric acid                          | 1¼       |    |

Although the present invention has been 45 described in connection with certain ingredients and certain proportions, it is not intended that such details shall be regarded as limitations upon the scope of the invention except in so far as they are included in the 50 accompanying claims.

## I claim:

1. A polish comprising water, mineral oil, wilkinite, abrasive earth, oxalic acid and tartaric acid in such proportions as to adapt it for use on automobile and other highly 55 polished surfaces.

2. A polish comprising water, mineral seal oil, a heavy oil, wilkinite, infusorial earth, oxalic acid and tartaric acid in such proportions as to adapt it for use on automobile and other highly 60 polished surfaces.

3. A polish comprising about 56 to 71% of water, 23 to 36% of mineral oil, 0.2 to 0.5% of wilkinite, 3 to 6% of infusorial earth, 1 to 1.5% of oxalic acid, and 1 to 1.5% of tar- 65

taric acid.

4. A polish comprising about 65% of water, 19% of mineral seal oil, 9½% of vis-

cous oil, ¼% of wilkinite, 3¾% of infu-

sorial earth, 1¼% of oxalic acid, and 1¼% 70

of tartaric acid.

In testimony whereof, I hereunto set my hand and seal this sixth day of April, 1927.

JAMES D. LINDSAY.

75

80

85

90

95

100